

July 2, 1940.

J. E. MARKEY

2,206,746

## METHOD OF PREPARING SKELP FOR WELDING

Filed Nov. 19, 1938

Fig. 1.



Fig. 2.



**INVENTOR**

INVENTOR  
*John E. Markey*

by his attorneys

Stebbins, Blanket Parmelee

## UNITED STATES PATENT OFFICE

2,206,746

METHOD OF PREPARING SKELP FOR  
WELDING

John E. Markey, Aliquippa, Pa., assignor to  
Jones & Laughlin Steel Corporation, Pittsburgh,  
Pa., a corporation of Pennsylvania

Application November 19, 1938, Serial No. 241,379

2 Claims. (Cl. 263—52)

This invention relates generally to the manufacture of welded pipe and, in particular, to the heating of skelp preparatory to the welding thereof.

In the manufacture of welded pipe according to the conventional method of heating skelp to welding temperature and drawing it through a welding bell or die, it has been found that the skelp tends to pick up the material composing the furnace bottom on which the skelp rests during heating. If the furnace is provided with a silica bottom, the material picked up therefrom adheres to the skelp in the form of silica scale and is a frequent cause for the rejection of pipe on inspection. Such rejections may amount to as high as 12% of the total production of a pipe mill. The loss represented by these rejections has caused considerable effort to be devoted to the problem without, so far as I am aware, achieving any satisfactory solution therefor.

I have invented a method and apparatus which are effective to reduce the percentage of rejections on account of silica scale to an almost negligible figure. I have discovered that the adherence to the skelp of the material composing the furnace bottom may be substantially prevented by appropriately controlling the temperature of the bottom. In a preferred practice of the invention I control the temperature of the furnace bottom in such manner as to maintain the temperature thereof below a certain value at which the material, e. g., silica, exhibits a tendency to adhere to the skelp when heated to welding temperature. My invention also contemplates a novel furnace construction adapted for the practice of the method above mentioned. An example of the furnace structure is illustrated in the accompanying drawing to which reference will be made for a complete explanation of my apparatus and method. In the drawing:

Fig. 1 is a section through a skelp heating furnace embodying the invention, taken on the plane slightly above the furnace bottom; and

Fig. 2 is a partial transverse section along the line II—II of Fig. 1; line I—I of Fig. 2 indicates the plane along which Fig. 1 is taken.

Referring now in detail to the drawing, a skelp heating furnace 10 comprises side walls 11, end walls 12, and a roof (not shown). The end walls are provided with suitable openings 13 through which skelp lengths 14 may be inserted and removed. The skelp lengths, while in the furnace, rest on the hearth or bottom thereof, indicated at 15. The furnace bottom is preferably com-

posed of a layer of sand 16 and a layer of gravel 17 supported on a foundation 18 of refractory brick or the like.

Cooling ducts 19, which may be simply suitable lengths of pipe of appropriate size, are embedded in the sand layer 16 with their ends open and protruding beyond the end walls 12, and are adapted, either by natural draft or forced circulation of air or other cooling fluid therethrough, to control the temperature of the furnace bottom. If natural draft through the ducts is relied on for cooling, the number and size of the ducts are so chosen that the resulting draft will have the desired cooling effect. In this case, the ducts will be connected by any suitable means (not shown) to an exhaust stack. If forced circulation of cooling fluid through the ducts is employed, the desired control over the temperature of the furnace body may be effected by varying the rate of fluid circulation. In this case, any known means such as fans, blowers, or the like, may be used to produce the desired circulation.

In practicing the invention with the aid of the apparatus described hereinabove, I deposit skelp lengths on the furnace bottom 15 for heating preparatory to passage through a welding bell or die. The furnace 10 may be heated in any convenient manner, e. g., by suitable fuel burners arranged therein in the known manner. The furnace is operated so that the skelp charged thereto will be heated to the welding temperature within the desired time. When the skelp has been properly heated, it is withdrawn from the furnace and passed through the welding die.

By means of the ducts 19, I so control the temperature of the furnace bottom as to maintain it below that at which silica scale from the material composing the furnace bottom adheres to the heated skelp and is picked up by the latter as it is withdrawn from the furnace for welding. The exact temperature of the bottom at which the skelp picks up silica scale is variable as it depends largely on local conditions. In any event, sufficient cooling can be had by the means shown to prevent almost entirely the objectionable adherence of silica experienced previously. In the typical furnace construction illustrated, I have found that for a furnace about 8' wide, eight 7" pipes arranged as shown in the drawing are sufficient to provide sufficient cooling by natural draft to reduce the objectionable adherence of silica scale to the skelp to an almost negligible amount.

By the aid of the invention, it has been possible

to reduce the percentage of pipe of a certain size rejected because of silica scale from about 12% to less than 1%. In another size, the rejections were reduced from about 6% to zero. In addition to reducing materially the number of rejections occasioned by silica scale, the invention prolongs the life of a furnace bottom considerably. By substantially eliminating the withdrawal of the material composing the furnace bottom 10 with the skelp, furnace bottoms last longer than heretofore and require renewal less often. The invention thus provides a relatively simple and inexpensive solution for the difficulty experienced heretofore with silica scale which, so far as I am 15 aware, has not previously been obtained despite numerous efforts extending over a substantial period of years.

Although I have illustrated and described but a preferred form and practice of the invention, 20 it will be understood that changes in the structure and procedure disclosed may be made without departing from the spirit of the invention or the scope of the appended claims.

I claim:

1. In a method of preparing skelp for welding to form pipe, the steps including providing a furnace bottom composed of granular silica, placing the skelp on said bottom, heating the skelp to welding temperature while on said bottom, and admitting cooling fluid to the interior of the mass of granular silica comprising the bottom, thereby cooling it to a temperature below that at which the granular silica forms a glaze on the 10 skelp.

2. The method of preventing the formation of silica scale on skelp in the manufacture of welded pipe wherein the skelp is heated to welding temperature in a furnace having a granular silica bottom, which method consists in maintaining said bottom at a temperature below that at which the silica of the bottom forms a glaze on the skelp, by circulating cooling fluid through the 15 silica bottom.

JOHN E. MARKEY.

20